

## UNITED STATES PATENT OFFICE

2,518,698

## CHEMICAL SENSITIZATION OF PHOTOGRAPHIC EMULSIONS

Wesley G. Lowe and Jean E. Jones, Rochester, N. Y., assignors to Eastman Kodak Company, Rochester, N. Y., a corporation of New Jersey

No Drawing. Application November 18, 1948, Serial No. 60,818

17 Claims. (Cl. 95—7)

1

This invention relates to photographic emulsions and more particularly to chemical sensitizers therefor.

It is well known that silver halide emulsions may be chemically sensitized with a variety of materials so as to increase the speed and generally the gamma of the emulsions as opposed to optical sensitizing in which the optical range of sensitivity is increased. Depending upon the materials and methods employed, it is generally regarded that chemical sensitization results in either the formation of silver sulfide on the surface of the silver halide crystal or results in the formation of small amounts of silver from the reduction of silver halide, which effect may be in addition to the former effect sometimes known as sulfur sensitizing. The present invention is concerned primarily with chemical sensitization apparently of the latter type.

Among the materials previously proposed for augmenting emulsion sensitivity may be mentioned basic compounds such as ammonia and certain aromatic and aliphatic amines such as triethylamine and triethanolamine; whereas other amines such as propylamylhexylamine are said to have no effect upon emulsion sensitivity. Similarly, we have found that simple polyamines such as ethylene diamine are not effective chemical sensitizers for silver halide emulsions. On the other hand, we have discovered certain polyamine compounds similar in structure to ethylene diamine which surprisingly are powerful sensitizers for silver halide emulsions.

One object of our invention is to provide chemically sensitized silver halide emulsions of enhanced sensitivity. Another object is to provide novel chemical sensitizing agents for photographic emulsions. Another object is to provide photographic emulsions having the sensitivity enhanced by means of both sulfur sensitizers and the novel sensitizers of our invention. A further object is to provide the methods of augmenting emulsion sensitivity utilizing the novel sensitizing agents. Another object is to provide photographic elements in which the novel emulsions are useful. Further objects of our invention will become apparent from consideration of the following description.

The objects of our invention are accomplished in part by the incorporation in silver halide emul-

2

sion layers of polyamine compounds such as diethylene triamine, triethylene tetramine or tetraethylene pentamine, tetrapropylene pentamine, and the like. The compounds have the general structure



where  $n$  is a positive integer from one to five, preferably one to three, and  $R$  is an alkylene chain of from two to four carbon atoms, preferably two carbon atoms. The three first-mentioned polyamines are particularly desirable not only because of the speed increases they effect, but also because their synthesis is relatively simple compared to polyamines of higher molecular weight, therefore they are more readily available in a high degree of purity.

The novel sensitizers are incorporated in the emulsions at any stage in their preparation but preferably before digestion is complete. Generally, in order to obtain the optimum sensitizing effect, we heat the emulsion after addition of the sensitizing agent. The sensitizers may be used in conjunction with other chemical and optical sensitizers such as the well known sulfur sensitizing compounds such as disclosed in Shepard U. S. Patents 1,574,944, granted March 2, 1926, and 1,623,499, granted April 5, 1927. Our novel sensitizers may be employed before, after or simultaneously with sulfur sensitizing. Also our novel sensitizers are useful with a variety of emulsions, producing pronounced speed increases in either negative or positive types of emulsions.

Our invention will now be illustrated by reference to the following specific examples.

Example 1

Several 100 cc. samples of a high speed bromo-iodide positive type of emulsion, each containing silver halide obtained from 20 grams of silver nitrate and peptized with a gelatin derivative by the process of the Lowe et al. U. S. application Serial No. 768,478, filed August 13, 1947, were adjusted to a pH of 6.0 and heated for 30 minutes at 50° C. with four mg. respectively of the diethylene triamine, triethylene tetramine and tetraethylene pentamine added in aqueous solution adjusted to pH 6.0. After this, each sample was added to 400 cc. of a five per cent gelatin solution and coated on a support and dried in the usual manner. After exposure of the emul-

sion coatings in an Eastman Type 2B Sensitometer, the samples were developed in a developer of the following composition:

Water, 1 liter  
p-Methylaminophenol sulfate, 0.3 gram  
Hydroquinone, 6.0 grams  
Sodium sulfite (dry), 38.0 grams  
Sodium bisulfite, 1.2 grams  
Sodium carbonate (dry), 19.0 grams  
Potassium bromide, 0.9 gram  
Citric acid, 0.7 gram

The exposed and processed emulsion coatings containing the polyamine sensitizers were found to have increased in speed as shown in the table following (samples A to D). 2B Sensitometers are described in J. Soc. Mot. Pict. Eng. 17 (1931) 536.

*Example 2*

100 cc. samples of the same type of positive emulsion used in the above examples were sulfur sensitized, e. g. with allyl thiourea as described in the Lowe et al., invention, adjusted to a pH of 6.0 and each heated for 30 minutes at 50° C. with four mg. of triethylene tetramine or tetraethylene pentamine added in aqueous solution adjusted to pH 6.0 with acetic acid. The samples were then coated, exposed and developed as in Example 1 and the characteristics of the resultant coatings are tabulated in the table following (samples G and H compared to F). It will be apparent from the data that appreciable speed increases have been effected by sensitizing the emulsions in the manner described.

*Example 3*

100 cc. samples of a high speed bromo-iodide negative type of emulsion containing silver halide from 26 grams of silver nitrate and 32 grams of gelatin were each diluted with water to 460 cc. and the pH adjusted to 6.4. To one sample was added one mg. of tetraethylene pentamine in aqueous solution adjusted to pH 7.0 with acetic acid. The emulsion and control sample were heated at 50° C. for one hour, then coated and dried as usual. The coatings were exposed on an Eastman Type 1B Sensitometer and developed four minutes in a developer of the following composition:

Water, about 125° F. (50° C.), 500 cc.  
p-Methylaminophenol sulfate, 2.2 grams  
Sodium sulfite, desiccated, 96.0 grams  
Hydroquinone, 8.8 grams  
Sodium carbonate, desiccated, 48.0 grams  
Potassium bromide, 5.0 grams  
Cold water to make, 1.0 liter

The character of the resultant emulsion is tabulated in the table following (samples I and J). Comparable results were obtained when the pentamine was heated with silver halide grains before addition of the gelatin.

*Example 4*

In the manner of Example 3, 460 cc. samples of the above negative type of emulsion containing gelatin were first sulfur sensitized by heating with a sulfur sensitizing agent at 59° C. for 20 minutes, then cooled to 40° C. and one or two mg. additions of the tetraethylene pentamine solution were added followed by heating at 50° C for 20 minutes. The samples were coated and dried as usual, exposed in an Eastman Type 1B Sensitometer and developed 4 minutes in the developer of Example 3. The characteristics of

the emulsions are shown in the table (samples J, K and L).

Similar speed increases were obtained by treatment of negative emulsions before or after sulfur sensitizing, with the other polyamines and salts thereof forming a part of our invention.

| Sample | Chemical Sensitizer  | Fog  | Gamma | (10/i) Speed |
|--------|----------------------|------|-------|--------------|
| 10     |                      |      |       |              |
| A      | None                 | 0.01 | 1.9   | 0.43         |
| B      | DET <sup>1</sup>     | 0.01 | 2.1   | 0.71         |
| C      | TET <sup>2</sup>     | 0.01 | 2.4   | 0.98         |
| D      | TEP <sup>3</sup>     | 0.01 | 2.4   | 1.0          |
| E      | Sulfur type          | 0.05 | 2.6   | 4.1          |
| F      | Sulfur and TET       | 0.05 | 3.0   | 5.4          |
| G      | do                   | 0.05 | 3.34  | 7.3          |
| H      | None                 | 0.03 | 0.34  | 7.6          |
| I      | TEP                  | 0.04 | 0.66  | 45.0         |
| J      | Sulfur type          | 0.13 | 1.50  | 650          |
| K      | Sulfur and 1 mg. TEP | 0.11 | 1.59  | 920          |
| L      | Sulfur and 2 mg. TEP | 0.13 | 1.46  | 960          |

<sup>1</sup> Diethylene triamine.

<sup>2</sup> Triethylene tetramine.

<sup>3</sup> Tetraethylene pentamine.

It will be apparent from consideration of the above data that the polyamines are effective in producing large speed increases in emulsions treated therewith, in most cases the increases with sulfur sensitized emulsions being considerably greater than obtained from the sensitizing effects of the individual sensitizers when used alone.

In the manner of the above examples, other types of silver halide emulsions may be treated with our novel sensitizing agents alone or in conjunction with other chemical or optical sensitizers. The amount of sensitizing agent may, depending upon the type of emulsion used, vary somewhat from the optimum amounts employed in the above examples, one-fifth to five times as much sensitizing agent producing emulsions of useful sensitivity. As is apparent, less heating is usually required when the larger amounts are employed and conversely when using the smaller quantities of sensitizing agent.

It will be noted in the above examples that the sensitizing of the emulsions with the novel compounds was effected at relatively low pH. This is not a limitation of our invention but more an advantage thereof since we are able to suppress sulfur sensitivity by lowering the pH of the emulsion and since the novel sensitizers are so active, further sensitization takes place even substantially below the neutral point when they are added to the emulsion.

The novel sensitizers may, in general, be employed in hydrophilic colloid emulsion vehicles; for example, gelatin, polyvinyl alcohol, partially hydrolyzed cellulose esters, such as cellulose acetate and co-polymers of polyvinyl alcohol. The sensitizers are suitable for the well known types of silver chloride, silver bromide and silver iodide emulsions and emulsions containing mixtures of these halides, containing the usual emulsion addenda such as antifoggants, spreading agents, coupler compounds, etc. Such emulsions are suitable to use in forming single as well as multilayer film useful in color photography which customarily include on a support two or more emulsion layers sensitized to different regions of the visible spectrum and may or may not contain coupler compounds. According to our invention such color films carry at least one emulsion layer containing a sulfide sensitizing agent of our invention.

Our invention having been described, we would have it understood that the preceding description

is by way of example only and that our invention is to be taken as limited only by the scope of the appended claims.

What we claim is:

1. A light-sensitive photographic emulsion comprising silver halide and a polyamine sensitizing agent having the general formula:



wherein R is an alkylene chain having from 2-4 carbon atoms and n is a positive integer of from 1-5.

2. A light-sensitive photographic emulsion comprising silver halide and a polyamine sensitizing agent selected from the group consisting of diethylene triamine, triethylene tetramine, tetraethylene pentamine, and their water-soluble salts of non-desensitizing acids.

3. A light-sensitive photographic emulsion comprising silver halide and triethylene tetramine as a sensitizing agent.

4. A light-sensitive photographic emulsion comprising silver halide and tetraethylene pentamine as a sensitizing agent.

5. A light-sensitive photographic emulsion comprising silver halide and diethylene triamine as a sensitizing agent.

6. A light-sensitive photographic emulsion comprising sulfur sensitized silver halide and triethylene tetramine as an additional sensitizing agent.

7. A light-sensitive photographic emulsion comprising sulfur sensitized silver halide and tetraethylene pentamine as an additional sensitizing agent.

8. A light-sensitive photographic emulsion comprising sulfur sensitized silver halide and diethylene triamine as an additional sensitizing agent.

9. The method of increasing the speed of a photographic silver halide emulsion which comprises imparting sulfur sensitivity to said emulsion and effecting a further increase in sensitivity by digestion of said emulsion in the presence of triethylene tetramine.

10. The method of increasing the speed of a photographic silver halide emulsion which comprises imparting sulfur sensitivity to said emulsion and effecting a further increase in sensitivity by digestion of said emulsion in the presence of tetraethylene pentamine.

11. The method of increasing the speed of a photographic silver halide emulsion which comprises imparting sulfur sensitivity to said emulsion and effecting a further increase in sensitivity

by digestion of said emulsion in the presence of diethylene triamine.

12. The method of sensitizing a photographic silver halide emulsion which comprises digesting said emulsion in the presence of a sulfur sensitizing agent and a polyamine sensitizing agent having the general formula:



10 wherein R is an alkylene chain having from 2-4 carbon atoms and n is a positive integer of from 1-5.

13. The method of sensitizing a photographic silver halide emulsion which comprises digesting said emulsion in the presence of a sulfur sensitizing agent and triethylene tetramine.

14. The method of sensitizing a photographic silver halide emulsion which comprises digesting said emulsion in the presence of a sulfur sensitizing agent and tetraethylene pentamine.

15. The method of sensitizing a photographic silver halide emulsion which comprises digesting said emulsion in the presence of a sulfur sensitizing agent and diethylene triamine.

16. A light-sensitive photographic emulsion comprising sulfur-sensitized silver halide and as an additional sensitizing agent a polyamine having the general formula



30 wherein R is an alkylene chain having from 2 to 4 carbon atoms and n is a positive integer of from 1 to 5.

17. The method of increasing the speed of a photographic silver halide emulsion which comprises imparting sulfur sensitivity to said emulsion, adjusting the pH of said emulsion to below neutrality, and effecting a further increase in sensitivity by digestion of said emulsion in the presence of a sensitizing agent having the general formula:



wherein R is an alkylene chain having from 2 to 4 carbon atoms and n is a positive integer of from 1 to 5.

WESLEY G. LOWE.  
JEAN E. JONES.

#### REFERENCES CITED

50 The following references are of record in the file of this patent:

#### FOREIGN PATENTS

| Number     | Country       | Date          |
|------------|---------------|---------------|
| 55 496,049 | Great Britain | Nov. 21, 1938 |

**Certificate of Correction**

August 15, 1950

Patent No. 2,518,698

WESLEY G. LOWE ET AL.

It is hereby certified that error appears in the printed specification of the above numbered patent requiring correction as follows:

Column 4, line 15, in the table, second column thereof, for "---- do -----" read *Sulfur and TEP*; and that the said Letters Patent should be read as corrected above, so that the same may conform to the record of the case in the Patent Office.

Signed and sealed this 7th day of November, A. D. 1950.

[SEAL]

THOMAS F. MURPHY,  
*Assistant Commissioner of Patents.*